



US010640914B2

(12) **United States Patent**  
**Hinks et al.**

(10) **Patent No.:** **US 10,640,914 B2**  
(45) **Date of Patent:** **May 5, 2020**

(54) **METHOD FOR DECOLORIZING TEXTILE MATERIALS**

|                   |        |                                 |
|-------------------|--------|---------------------------------|
| 7,192,988 B2      | 3/2007 | Smith et al.                    |
| 7,959,807 B2      | 6/2011 | Mukai et al.                    |
| 2003/0056296 A1 * | 3/2003 | Hirsch ..... C09B 67/0096 8/102 |

(71) Applicant: **NORTH CAROLINA STATE UNIVERSITY**, Raleigh, NC (US)

|                 |         |                 |
|-----------------|---------|-----------------|
| 2005/0028291 A1 | 2/2005  | Bechtold et al. |
| 2005/0115004 A1 | 6/2005  | Tashiro et al.  |
| 2006/0230541 A1 | 10/2006 | Hirsch et al.   |
| 2008/0255259 A1 | 10/2008 | Ozer et al.     |
| 2010/0281623 A1 | 11/2010 | Oshel et al.    |
| 2012/0125844 A1 | 5/2012  | Dongare et al.  |
| 2015/0059103 A1 | 3/2015  | Liu et al.      |

(72) Inventors: **David Hinks**, Apex, NC (US); **Guan Wang**, Raleigh, NC (US); **Xiuzhu Fei**, Raleigh, NC (US); **Harold Freeman**, Raleigh, NC (US)

(73) Assignee: **North Carolina State University**, Raleigh, NC (US)

FOREIGN PATENT DOCUMENTS

|    |               |        |
|----|---------------|--------|
| CN | 101195968 B   | 6/2008 |
| CN | 101215776 A   | 7/2008 |
| CN | 101967761 A   | 2/2011 |
| CN | 104805720 A   | 7/2015 |
| WO | 2014047620 A1 | 3/2014 |

(\*) Notice: Subject to any disclaimer, the term of this patent is extended or adjusted under 35 U.S.C. 154(b) by 0 days.

(21) Appl. No.: **15/928,136**

OTHER PUBLICATIONS

(22) Filed: **Mar. 22, 2018**

International Search Report, PCT/US2016/052593, dated Jan. 5, 2017.

(65) **Prior Publication Data**

International Search Report, PCT/US2016/047303, dated Nov. 21, 2016.

US 2018/0209089 A1 Jul. 26, 2018

Chu, Wei et al.; "Photo-sensitization of diazo disperse dye in aqueous acetone", Chemosphere, (1999). vol. 39, No. 10, pp. 1667-1677.

**Related U.S. Application Data**

Prola, Lizzie D.T. et al.; "Comparison of Jatropha curcas shells in natural form and treated by non-thermal plasma as biosorbents for removal of reactive Red 120 textile dye from aqueous solution", Industrial Crops and Products, vol. 46, pp. 328-340, 2013.

(63) Continuation of application No. PCT/US2016/052593, filed on Sep. 20, 2016.

Khadhraoui, M. et al.; "Discoloration and detoxification of a Congo red dye solution by means of ozone treatment for a possible water reuse", Journal of Hazardous Materials, vol. 161, pp. 974-981, 2009.

(51) **Int. Cl.**

Szpyrkowicz, L. et al.; "A Comparative Study on Oxidation of Disperse Dyes by Electrochemical Process, Ozone, Hypochlorite and Fenton Reagent", Water Research 2001, vol. 35, No. 9, pp. 2129-2136.

**D06L 4/30** (2017.01)  
**D06P 5/13** (2006.01)  
**D06P 1/651** (2006.01)  
**D06P 1/62** (2006.01)  
**D06L 4/70** (2017.01)

Neamtu, M. et al.; "Decolorization of disperse red 354 azo dye in water by several oxidation processes—a comparative study", Dyes and Pigments 60 (2004) 61-68.

(52) **U.S. Cl.**

(Continued)

CPC ..... **D06L 4/30** (2017.01); **D06L 4/70** (2017.01); **D06P 1/621** (2013.01); **D06P 1/65112** (2013.01); **D06P 5/134** (2013.01)

(58) **Field of Classification Search**

Primary Examiner — Eisa B Elhilo  
(74) Attorney, Agent, or Firm — Womble Bond Dickinson (US) LLP

CPC ... D06L 4/30; D06L 4/70; D06P 5/134; D06P 5/155; D06P 1/65112

See application file for complete search history.

(56) **References Cited**

**ABSTRACT**

U.S. PATENT DOCUMENTS

The disclosure relates to a method for decolorization of a dye-colored synthetic polymer, which includes the steps of treating a dye-colored synthetic polymer, such as polyester, with a treatment composition at pH 6 or less, the treatment composition comprising sodium formaldehyde sulfoxylate, water, and a ketone. The resulting decolorized synthetic polymer is then separated from the treatment composition.

|               |         |                          |
|---------------|---------|--------------------------|
| 5,366,510 A   | 11/1994 | Wasinger et al.          |
| 5,613,983 A   | 3/1997  | Terry et al.             |
| 5,711,764 A * | 1/1998  | Wasinger ..... D06L 1/06 |
|               |         | 510/276                  |
| 5,989,296 A   | 11/1999 | Patton et al.            |
| 6,120,554 A   | 9/2000  | Patton et al.            |
| 6,217,621 B1  | 4/2001  | Modebelu et al.          |

**20 Claims, No Drawings**

(56)

**References Cited****OTHER PUBLICATIONS**

- Arslan, I; "Treatability of a simulated disperse dye-bath by ferrous iron coagulation, ozonation, and ferrous iron-catalyzed ozonation", Journal of Hazardous Materials B85 (2001) 229-241.
- Yang, Y.Q. et al.; "Decolorization of dyes using UV/H<sub>2</sub>O<sub>2</sub> photochemical oxidation", Textile Chemist and Colorist (1998) vol. 30, 4, 27-35.
- Kim, Tak-Hyun et al.; "Comparison of disperse and reactive dye removals by chemical coagulation and Fenton oxidation", Journal of Hazardous Materials B112 (2004) 95-103.
- Hsing, Hao-Jan et al.; "The decolorization and mineralization of Acid Orange 6 azo dye in aqueous solution by advanced oxidation processes: A comparative study", Journal of Hazardous Materials 141 (2007) 8-16.
- Surpateanu, M.; et al.; "Advanced oxidation processes for decolorization of aqueous solution containing Acid Red G azo dye", Central European Journal of Chemistry 2(4) (2004), 573-588.
- Salazar, R. et al.; "Finding the best Fe<sup>2+</sup>/Cu<sup>2+</sup> combination for the solar photoelectro-Fenton treatment of simulated wastewater containing the industrial textile dye Disperse Blue 3", Applied Catalysis B: Environmental 115-116 (2012) 107-116.
- He, Y. et al.; "Fenton oxidation of 2,4- and 2,6-dinitrotoluene and acetone inhibition", Frontiers of Environmental Science & Engineering in China, Sep. 2008, vol. 2, Issue 3, pp. 326-332.
- Ciner, F. et al.; "Treatability of Dye Solutions Containing Disperse Dyes by Fenton and Fenton-Solar Light Oxidation Processes", CLEAN Soil Air Water 2013, 41(1), 80-86.
- Kumar, D.; "Use of Photo-Fenton Reagent for the Degradation of Thioglycolic Acid", International Journal of Analytical, Pharmaceutical and Biomedical Sciences, 2014, 3(3), 1-5.
- Barbusinski, K.; "Fenton Reaction—Controversy Concerning the Chemistry", Ecological Chemistry and Engineering, 2009, 16, 3, 347-358.
- Bigda, R.; "Fenton's Chemistry: An Effective Advanced Oxidation Process", environmental Technology May/Jun. 1996, 35-39.
- Prato-Garcia, D. et al.; "Degradation of azo dye mixtures through sequential hybrid systems: Evaluation of three advanced oxidation processes for the pre-treatment stage", Journal of Photochemistry.
- De Amorim, C. et al.; "Comparison of various advanced oxidation processes for azo dye degradation", Engenharia Sanitaria E Ambiental, Oct.-Dec. 2009, 14, 4, 543-550.

\* cited by examiner

## 1

## METHOD FOR DECOLORIZING TEXTILE MATERIALS

## CROSS-REFERENCE TO RELATED APPLICATIONS

This application is a continuation of International App. No. PCT/US2016/052593; filed Sep. 20, 2016, which International Application was published by the International Bureau in English on Mar. 30, 2017, and claims priority to U.S. Provisional Application No. 62/222,993, filed Sep. 24, 2015, each of which is incorporated by reference in their entirety and for all purposes.

## FIELD OF THE INVENTION

The present disclosure relates to methods for decolorization of dye-colored synthetic polymer materials, particularly polyester-containing textiles.

## BACKGROUND OF THE INVENTION

In our increasingly waste-conscious world, tremendous strides have been made with respect to recycling synthetic materials. Significant progress has been made, in particular, in the area of polyester products, such as polyethylene terephthalate (PET) products. Total global tonnage of such products is in the tens of millions, primarily in the form of textiles and packaging (e.g., PET bottles). Recycling and reuse of the polymer material in PET bottles has become particularly widespread, and such recycling processes typically include mechanical processing techniques that produce polymer chips that can be used as a feedstock in a variety of polyester product manufacturing processes including those used to make textiles.

However, use of recycling techniques for synthetic fiber products such as textiles has not reached the same level of widespread acceptance. One problem associated with synthetic fiber recycling is the fact that virtually all synthetic fibers are colored as part of the manufacturing process. Although many thermoplastic fibers can be melted and either extruded or injection molded into new products, the presence of colorant in the polymer material reduces the commercial attractiveness of many synthetic textile materials otherwise available for recycle and reuse.

Certain recycling processes have been proposed for polyester materials that includes dye removal steps. See, for example, U.S. Pat. No. 7,192,988 to Smith et al. and U.S. Pat. No. 7,959,807 to Mukai et al. However, both of the above-noted patents also suggest depolymerization and repolymerization steps, which greatly increase the cost and complexity of those processes.

## DETAILED DESCRIPTION

As stated above, previous efforts to recycle dye-colored polymers required depolymerization and repolymerization steps, which greatly increase the cost and complexity of those processes. There remains a need in the art for a method for decolorizing polymer materials which does not require destroying or significantly degrading the structure of the polymer.

Although considerable research has focused on removal of colorants from wastewater streams such as those associated with textile plants, relatively little research has been conducted on selectively removing colorant from polymer materials, which presents challenges not present in waste-

## 2

water treatment. Processes used for wastewater treatment are generally intended to, and are effective in, breaking down or removing many more compounds from water than just colorants. While the general removal or break-down of organic compounds is appropriate and desirable for the purposes of wastewater cleanup, these processes often are not sufficiently efficient in selectively removing colorants and can result in the removal or break-down of the synthetic polymers themselves. In batch processes which employ reagents at pre-determined concentrations for controlled periods of time, these processes can remove or destroy any reagents along with colorants.

The present disclosure provides a method of decolorizing synthetic polymer materials such as synthetic polymer-containing textiles without causing significant degradation of the structure of the polymers. The method is particularly well-suited for polyester-containing textiles, although the method can be applied to textiles containing other synthetic polymers. The method involves treating the synthetic polymer with sodium formaldehyde sulfoxylate (SFS) ( $\text{NaHSO}_2\text{CH}_2\text{O}_2\text{H}_2\text{O}$ ). It has been found that SFS can be effective in decolorizing dye-colored polymeric materials. Although not bound by a theory of operation, SFS is believed to release a reducing radical according to the mechanisms set forth in the two equations below.



Unexpectedly, when treating dye-colored synthetic polymers, it has been found that the addition of a ketone such as acetone to the treatment increases the efficacy of the decolorizing treatment such that significant decolorization of synthetic polymers occurs over reasonable time periods and under conditions which are amenable to manufacturing. The addition of the ketone to the treatment has not been found to significantly degrade synthetic polymers during the treatment. In fact, it has been found that it is possible to use this treatment to decolorize textiles formed from synthetic polymers, and that the decolorized textiles can then be recycled, for example by re-using and re-dying the polymers.

It is surprising that combining a ketone with SFS under these conditions has this effect. It was expected that the SFS would break down the ketone along with the colorants, and/or that the presence of the ketone would have inhibited the effectiveness of the SFS. However, the opposite has been found to occur: addition of the ketone to the SFS in the disclosed treatment increases, rather than inhibits, the effectiveness of the treatment in breaking down colorants. Additionally, this combined treatment has been found to have little if any detrimental effect on the structure of the synthetic polymer. Without being bound by theory, it is believed that the presence of the ketone may at least partially dissolve the dye, and/or may at least partially swell the polymer material so that the dye is more easily extracted from the polymer. Alternatively or in addition, this dissolution and/or swelling may allow better contact between the components of the SFS and the dye, thus increasing the effectiveness of the decolorizing treatment.

The method for decolorizing a dye-colored synthetic polymer comprises treating a dye-colored synthetic polymer with a treatment composition, the treatment composition

comprising (a) SFS, (b) water, and (c) a ketone dissolved in the treatment composition; wherein the treatment composition has a pH of 6 or less, and the treating is carried out at a temperature of at least 50° C. and for a duration of time sufficient to at least partially decolorize the synthetic polymer; and following the treating, separating at least partially decolorized synthetic polymer from the treatment composition. In one example, the treatment composition comprises from 2.5 g/L to 50 g/L of SFS.

The ketone of the treatment composition can comprises a ketone selected from the group consisting of acetone, methyl ethyl ketone, 2-pentanone, 3-pentanone, 2-hexanone, 3-hexanone, methyl isobutyl ketone, methyl n-propyl ketone, methyl isopropyl ketone, ethyl ketone, and any combination thereof. In one example, the ketone of the treatment composition comprises acetone. In another example, the ketone of the treatment composition consists essentially of acetone.

In one example, a weight ratio of the water to the ketone in the treatment composition is from 4:1 to 1:4. In another example, the weight ratio of the water to the ketone is from 2:1 to 1:2.

The treatment composition can be held at a constant temperature during the treating step, or can be varied over the course of the treating step. The temperature of the treatment composition can be at least 70° C. The temperature of the treating composition during the treating step can be from 50° C. to 140° C. The temperature of the treating composition during the treating step can be from 70° C. to 120° C. The temperature of the treating composition during the treating step can be from 80° C. to 110° C. The temperature of the treating composition during the treating step can be about 100° C.

During the treating step, the liquor ratio present, i.e., the ratio of the weight of the treatment composition to the weight of the textile being treated, can be at least 10:1. In one example, the liquor ratio present during the treating step is at least 20:1.

The dye-colored synthetic polymer can be colored with a dye selected from the group consisting of acid dyes, basic dyes, mordant dyes, direct dyes, sulfur dyes, disperse dyes, reactive dyes, and vat dyes.

The dye-colored synthetic polymer can be colored with a dye selected from the group consisting of acridine dyes, anthraquinone dyes, arylmethane dyes, azo dyes, cyanine dyes, nitro dyes, nitroso dyes, phthalocyanine dyes, quinone dyes, thiazine dyes, thiazole dyes, xanthene dyes, fluorene dyes, stilbene dyes, vinyl sulfone dyes, triazine dyes, sulfur dyes, indigoid dyes, and any combination thereof. In one example, the dye-colored synthetic polymer is colored with a cationic dye. In a particular example of the method, the dye-colored synthetic polymer is colored with an azo dye, an anthraquinone dye, or any combination thereof.

The synthetic polymer can comprise a polymer selected from the group consisting of regenerated celluloses, polyesters, polyamides, polyurethanes, polyolefins, acrylonitriles, and any combination thereof. In one example, the synthetic polymer comprises polyethylene terephthalate (PET). In another example, the synthetic polymer consists essentially of polyethylene terephthalate (PET).

The dye-colored synthetic polymer can be present in the form of a dye-colored synthetic polymer-containing textile. The textile can be a woven textile, a knit textile, a braided textile, or a non-woven textile.

The effectiveness of the present decolorization method can be determined using various quantitative methods known to those of skill in the art. In one example, wherein

the dye-colored synthetic polymer comprises a dye-colored synthetic polymer textile, following the treating, the at least partially decolorized textile material has a K/S value of less than 3, as determined using equation (i):

$$K/S = \frac{(1 - R)^2}{2R} \quad (i)$$

wherein R=1.0 at 100% reflectance.

In another example, following the treating, the at least partially decolorized synthetic polymer textile has a K/S value as determined using equation (i) which is at least 70% lower than the K/S value of the dye-colored synthetic polymer textile prior to the treating.

The degree of degradation caused to the synthetic polymer by the treatment can be evaluated using various quantitative methods known to those of skill in the art. In one example, a difference between an intrinsic viscosity of the synthetic polymer before and after the treating is less than plus or minus 5%. In another example, a difference between the viscosity average molecular weight of the synthetic polymer before and after the treatment is less than plus or minus 2%. In yet another example, a difference between the viscosity average molecular weight of the synthetic polymer before and after the treatment is less than plus or minus 1%.

The method can further comprise a step of presoaking the dye-colored synthetic polymer prior to the treating, wherein the pre-soak composition comprises an aqueous solution of an organic solvent. In one example, the organic solvent of the pre-soak composition comprises a ketone. In another example, the organic solvent of the pre-soak composition comprises the same ketone as the treatment composition. In yet another example, the organic solvent of the pre-soak composition comprises acetone. In a particular example, the organic solvent of the pre-soak solution consists essentially of acetone. The pre-soak composition can be effective to at least partially swell the dye-colored synthetic polymer.

The method for decolorizing a dye-colored synthetic polymer can be a method for decolorizing a dye-colored polyethylene terephthalate-containing textile, comprising the steps of optionally pre-soaking a dye-colored polyethylene terephthalate-containing textile in a presoak composition comprising water and acetone; treating the dye-colored textile with a treatment composition, the treatment composition comprising (a) from of SFS, (b) water, and (c) acetone; wherein the treatment composition has a pH of 6 or less, and the treating is carried out at a temperature of at least 70° C. and for a duration of time sufficient to at least partially decolorize the dye-colored textile; and following the treating, separating at least partially decolorized textile from the treatment composition.

These and other features, aspects, and advantages of the disclosure will be apparent from a reading of the following detailed description. The invention includes any combination of two, three, four, or more of the above-noted embodiments as well as combinations of any two, three, four, or more features or elements set forth in this disclosure, regardless of whether such features or elements are expressly combined in a specific embodiment description herein. This disclosure is intended to be read holistically such that any separable features or elements of the disclosed invention, in any of its various aspects and embodiments, should be viewed as intended to be combinable unless the context clearly dictates otherwise.

The present disclosure will now be described more fully hereinafter with reference to exemplary embodiments thereof. These exemplary embodiments are described so that this disclosure will be thorough and complete, and will fully convey the scope of the disclosure to those skilled in the art. Indeed, the disclosure may be embodied in many different forms and should not be construed as limited to the embodiments set forth herein; rather, these embodiments are provided so that this disclosure will satisfy applicable legal requirements. As used in the specification, and in the appended claims, the singular forms "a", "an", "the", include plural variations unless the context clearly dictates otherwise.

The present disclosure provides a method for decolorization of a dye-colored synthetic polymer without requiring depolymerization of its polymeric structure. The process is particularly advantageous for treating textile materials intended to be recycled as removal or diminution of colorant within the textile material can increase the value of the recycled material. The method generally includes the step of treating a dye-colored synthetic polymer with a solution comprising (a) SFS, (b) water, and (c) a ketone dissolved in the treatment composition; wherein the treatment composition has a pH of 6 or less.

The dye-colored synthetic polymer to be treated can be colored with various types of dyes. Exemplary types of dyes include acid dyes, basic dyes, mordant dyes, direct dyes, sulfur dyes, disperse dyes, reactive dyes, and vat dyes. Dyes can also be characterized by the chemical structure of the chromophore or reactive portion of the dye molecule, with examples including acridine, anthraquinone, arylmethane (including di- and triarylmethane), azo (including monoazo, diazo and triazo dyes), cyanine, nitro, nitroso, phthalocyanine, quinone (e.g., azin, indamin, indophenol, oxazin, oxazine), thiazine, thiazole, xanthene, fluorene, stilbene, vinyl sulfone, triazine, sulfur, and indigoid. Synthetic polymers such as polyester material colored with reactive dyes, basic dyes, acid dyes, or disperse dyes are particularly well-suited for use with the present method, including materials dyed with azo, nitro, quinoline, or anthraquinone dyes.

The overall amount of SFS will vary depending on the type of dye to be decolorized, the amount of dye present in the dye-colored synthetic polymer, the desired level of decolorization, and the material to be treated. The concentration of SFS can be at least 2.5 g/L, or at least 5 g/L, or at least 10 g/L. A typical range of SFS concentration is from 2.5 g/L to 50 g/L (e.g., 25 to 45 g/L).

In accordance with the present method, the presence of both water and a ketone which is soluble in the treatment composition is important for significant decolorization of the synthetic polymer. It has been found that the use of treatment compositions without the ketone do not significantly reduce coloration in certain synthetic polymer materials under the general conditions discussed herein. Although not bound by any particular theory of operation, it is believed that the presence of the ketone enhances decolorization by dissolving at least a portion of the dye and/or swelling at least a portion of the synthetic polymer and, thus, bringing some portion of the dye material into better contact with the treatment composition. In other words, the ketone may cause release of at least a portion of the dye from the fibrous mass of the textile and/or may cause swelling of at least some of the fibers of the textile so that the treatment composition has better access to the dye molecule.

Although acetone is a particularly advantageous choice, other ketones or combinations of ketones could also be used in certain embodiments. Examples of other ketones include

methyl ethyl ketone, 2-pentanone, 3-pentanone, 2-hexanone, 3-hexanone, methyl isobutyl ketone, methyl n-propyl ketone, methyl isopropyl ketone, ethyl ketone, and combinations thereof. The selection of ketone will depend, in part, on the type of synthetic polymer and the chemical nature of the dye to be removed therefrom. Considerations for ketone selection include the stability/inertness of the solvent in the presence of the SFS and the level of solubility of the dye in the ketone.

10 The relative amounts of the water to the ketone can vary and will depend, in part, on the level of decolorization required, the type of synthetic polymer to be decolorized, and the type and structure of the dye. The weight ratio of the water to the ketone can be from 4:1 to 1:4, such as from 2:1 15 to 1:2 (e.g., about 1:1). The ketone will typically be present in an amount of at least about 10% by total weight of the water and ketone portion of the treatment composition, more typically at least 20% or at least 30% or at least 40% of the total weight of water and ketone in the treatment composition.

20 The treatment method involves contacting the dye-colored synthetic polymer to be treated with the treatment composition under conditions sufficient to cause decolorization to occur. The treatment process will typically entail combining the dye-colored synthetic polymer with the treatment composition in a suitable vessel, optionally equipped for stirring or agitation during the treatment process. The vessel is also advantageously equipped to heat the synthetic polymer and treatment composition during the treatment period.

25 Parameters of the treatment process such as time, pH, temperature, pressure, and liquor ratio can vary and will depend, in part, on the exact composition of the treatment composition, the desired level of decolorization, other treatment parameters (e.g., the time and temperature of the treatment process can vary inversely), and the type of synthetic polymer and dye to be treated. The time during which the synthetic polymer is exposed to the treatment composition will typically be at least 5 minutes, or at least 30 30 minutes, or at least 20 minutes. Significant decolorization is typically accomplished with treatment times of no more than about 120 minutes, such as no more than 90 minutes, or no more than 60 minutes. An exemplary treatment range is from 15 minutes to 75 minutes.

35 The treatment temperature will typically range from room temperature to about 150° C., with an advantageous range of from 60° C. to 120° C. In certain embodiments, elevated temperatures, such as a temperature of at least 100° C. or at least 110° C., provide the best decolorization results. The treatment process is typically conducted at atmospheric pressure, although higher pressures could be used with the present method.

40 The pH of the treatment composition is typically in the acidic range, with an exemplary pH range of about 1 to about 55 6 (e.g., from 2 to 5). The pH is typically below about 6, or below about 5.

45 The liquor ratio (L.R.) during treatment, which is defined as the ratio of the weight of the treatment composition to the weight of the textile being treated, is typically at least 5:1, or at least 10:1, or at least 20:1. In certain embodiments, the liquor ratio is from 5:1 to 60:1 (e.g., from 10:1 to 50:1).

50 Although the treatment process can be accomplished by treating the synthetic polymer (e.g., textile material) with the treatment composition in a single step, it can be advantageous to presoak the synthetic polymer in a pre-soak composition of an aqueous solution of an organic solvent (e.g., water and a lower alcohol or water and acetone) for a period

of time prior to treatment with the treatment composition. Although not bound by any particular theory of operation, it is believed that pre-treatment of the synthetic polymer with the pre-soak composition may allow dissolution of a larger percentage of the dye and/or greater swelling of the synthetic polymer, which can enhance the effectiveness of decolorizing treatment. The pre-soaking step can be accomplished over a variable time period, but typically pre-soaking occurs for at least 5 minutes, or at least 10 minutes, or at least 15 minutes. Note that the temperature of the pre-soaking step can be lower than the treatment temperature. For example, pre-soaking can occur at room temperature or a temperature no higher than about 60° C., whereas the decolorizing treatment can be higher, such as greater than 100° C. as noted above.

In one particularly advantageous example, the treatment process is applied to a dyed polyester material and the treatment composition comprises the SFS in a water/acetone mixture (e.g., at a weight ratio of water to acetone of about 2:1 to about 1:2).

As used herein, reference to "decoloring," "decolorized" or "decolorization" refers to the reduction or elimination of the primary color associated with a particular colorant and refers, in particular, to degradation of the chromophore portion of a colorant molecule responsible for its color. The extent of decolorization of the synthetic polymer using the treatment process disclosed herein can be determined by visual inspection or quantified by correlating reflectance with dye concentration. Kubelka developed numerous formulas for correlating reflectance with concentration by making scattering and surface difference corrections. See, generally, Paul Kubelka, Franz Munk, Ein Beitrag zur Optik der Farbanstriche, Zeits. f. Techn. Physik 1931; 12:593-601. It has been determined that the ratio of light absorption to light scattering at a given wavelength is proportional to the concentration of the dye in the sample. The theory works best for optically thick materials. The relationship shown below is derived from the Kubelka-Munk equation.

$$K/S = \frac{(1 - R)^2}{2R}$$

wherein R=1.0 at 100% reflectance, K is the absorption coefficient, and S is the scattering coefficient. Color strength is defined as:

$$\text{Color strength} = [(K/S)_{\text{batch}} / (K/S)_{\text{standard}}] \times 100.$$

Accordingly, decolorization of textile materials using the present invention can be characterized by reference to a change in K/S value, with a reduction in the K/S value indicating a reduction in dye color. In certain examples, the decolorization process of the invention can result in a K/S value of less than 3, such as less than 2.5 or less than 2.0. In certain examples, the K/S value following treatment will be less than 1.5 or less than 1.0 (e.g., from 0.1 to 1.5). The decolorization effect of the method can also be characterized as a percentage reduction of K/S value by comparing the K/S value of the untreated textile and the K/S value following treatment. In certain examples, the K/S value is reduced by the treatment process of the invention by at least 25%, but in any many advantageous examples, the percentage reduction in K/S values is at least 60%, at least 70%, at least 80%, at least 90%, or at least 95%.

The treatment process of the method is also advantageous in that the treatment accomplishes significant decolorization

without significant degradation of the polymer structure of the synthetic polymer. Changes in polymer structure can be assessed by determining changes in intrinsic viscosity and viscosity average molecular weight of the decolorized textile material. In certain advantageous examples, the intrinsic viscosity, viscosity average molecular weight, and degree of polymerization (DP) of the treated textile material is substantially unchanged by the treatment process. For example, it is preferable for the intrinsic viscosity, molecular weight, and DP of the treated synthetic polymer to be within 3% (e.g., within 2% or within 1%) of the same value for the synthetic polymer prior to treatment.

The relative viscosity (RV) of a polymer can be obtained by comparing the drop time (T) of a PET solution with the drop time ( $T_0$ ) of the pure solvent itself:  $RV = T/T_0$ . The intrinsic viscosity ( $[\eta]$ ) of the material is calculated using the equation:  $[\eta] = [(RV - 1) \times 0.6907] + 0.0631$ . Degree of polymerization (DP) can be calculated by the Mark-Houwink equation:  $[\eta] = KM^a$ , where  $[\eta]$  is the polymer intrinsic viscosity and M is the viscosity average molecular weight. The parameters, a and K, depend on the particular polymer-solvent system. See, generally, Brandup, J.; Immergut, E. H. Polymer Handbook, 3rd ed.; Wiley: New York, 1989; Chapter VII: 23.

## EXAMPLES

### Example 1

Several experiments were conducted to determine effectiveness of decolorization using different solvent ratios, treatment temperatures, liquor ratios, and SFS concentrations. The experiments were performed on cationic dyeable polyester (PET) fabric samples. For each experiment, a treatment time of 40 minutes was used. Table 1 below sets forth the four factors that were modified for each experiment. Experiments were conducted using every combination of the factors of Table 1 (e.g., a SFS concentration of 5 g/L at both 100° C. and 110° C., both L.R. ratios at 110° C., and the like).

TABLE 1

| Factor        | Low level | High level |
|---------------|-----------|------------|
| [SFS]         | 5 g/L     | 20 g/L     |
| Temperature   | 100° C.   | 110° C.    |
| L.R.          | 30        | 50         |
| Water:Acetone | 1:1       | 1:2        |

All experiments resulted in significant decolorization of the polyester. One of the most effective combinations was a SFS concentration of 20 g/L, a water:acetone ratio of 1:2, a L.R. of 30, and a temperature of 100° C.

The samples treated for 30 minutes gave color removal results comparable to the longer treatment time. Although increasing the amount of acetone causes an increase in the amount of dyes that can be extracted from the fabric, when the percentage of organic solvent is too high, the solubility of the reducing agent decreases and decolorization performance decreases. When the concentration of SFS is at the lower tested level (5 g/L), the performance was better than that at the higher level (20 g/L).

### Example 2

PET fabric samples dyed with an azo dye (Orange 30), an anthraquinone dye (Blue 60), and a quinoline dye (Yellow

54) were selected. A decolorization treatment using SFS as a reducing agent was applied to each fabric sample using the conditions set forth in Table 2 below.

In sample whiteness test after treatment, K/S values were measured. For each dye, the SFS treatment was successful in reducing coloration. For the Orange 30 dye, the K/S value prior to treatment was 31.778 and the value after treatment was 1.765 for the Blue 60 dye, the K/S value before treatment was 15.121 and the value after was 2.4. For the Yellow 54 dye, the K/S before treatment was 26.353 and the value after was 6.438. The data suggested that the SFS treatment is more effective for the azo and anthraquinone dyes as compared to the quinoline dye.

TABLE 2

|            |         |
|------------|---------|
| Fabric Wt. | 1 g     |
| SFS        | 40 g/L  |
| Acetone    | 50 mL   |
| Water      | 50 mL   |
| T          | 100° C. |
| pH         | 4.5     |
| t          | 60 min  |

## Example 3

A PET fabric sample (2 g) was treated in the same manner as generally described in Example 2 above. The relative viscosity of the PET polymer was measured using an Ubbelohde viscometer with o-chlorophenol as solvent. The resulting relative viscosity was compared to a 2 g untreated prescoured PET fabric.

For the viscosity test, all fabric samples were dissolved in 20 mL solvent at a temperature of 76.5° C. for 40 min. The solution was cooled and placed in an Ubbelohde viscometer. Using the relative viscosity measurement, the DP of each sample was calculated using the Mark-Houwink equation, wherein  $a=1.7 \times 10^{-4}$  and  $K=0.83$ . The resulting IV and viscosity average MW for each sample are set forth in Table 3 below. As noted therein, the decolorization treatment did not significantly affect the integrity of the polymer material.

TABLE 3

| Fabric Type   | IV (dL/g) | MW    |
|---------------|-----------|-------|
| Untreated     | 0.5024    | 19425 |
| SFS Treatment | 0.5002    | 19349 |

The present invention provides for the following clauses, the numbering of which is not to be construed as designating levels of importance.

Clause 1: A method for decolorizing a dye-colored synthetic polymer, comprising:

treating a dye-colored synthetic polymer with a treatment composition, the treatment composition comprising  
 (a) sodium formaldehyde sulfoxylate,  
 (b) water, and  
 (d) a ketone dissolved in the treatment composition; wherein the treatment composition has a pH of 6 or less, and the treating is carried out at a temperature of at least 50° C. and for a duration of time sufficient to at least partially decolorize the synthetic polymer; and  
 following the treating, separating at least partially decolorized synthetic polymer from the treatment composition.

Clause 2: The method of Clause 1, wherein the treatment composition comprises from 2.5 g/L to 50 g/L of sodium formaldehyde sulfoxylate.

Clause 3: The method of any preceding Clause, wherein the ketone comprises a ketone selected from the group consisting of acetone, methyl ethyl ketone, 2-pentanone, 3-pentanone, 2-hexanone, 3-hexanone, methyl isobutyl ketone, methyl n-propyl ketone, methyl isopropyl ketone, ethyl ketone, and any combination thereof.

Clause 4: The method of any preceding Clause, wherein the ketone comprises acetone.

Clause 5: The method of any preceding Clause, wherein the ketone consists essentially of acetone.

Clause 6: The method of any previous Clause, wherein a weight ratio of the water to the ketone in the treatment composition is from 4:1 to 1:4.

Clause 7: The method of Clause 1, wherein the treating is carried out at a temperature of at least 70° C.

Clause 8: The method of any preceding Clause, wherein a liquor ratio present during the treating step is at least 10:1.

Clause 9: The method of any preceding Clause, wherein the dye-colored synthetic polymer is colored with a dye selected from the group consisting of acid dyes, basic dyes, mordant dyes, direct dyes, sulfur dyes, disperse dyes, reactive dyes, and vat dyes.

Clause 10: The method of any preceding Clause, wherein the dye-colored synthetic polymer is colored with a dye selected from the group consisting of acridine dyes, anthraquinone dyes, arylmethane dyes, azo dyes, cyanine dyes, nitro dyes, nitroso dyes, phthalocyanine dyes, quinone dyes, thiazine dyes, thiazole dyes, xanthene dyes, fluorene dyes, stilbene dyes, vinyl sulfone dyes, triazine dyes, sulfur dyes, indigoid dyes, and any combination thereof.

Clause 11: The method of any preceding Clause, wherein the dye-colored synthetic polymer material is colored with an azo dye, an anthraquinone dye, or any combination thereof.

Clause 12: The method of any preceding Clause, wherein the synthetic polymer comprises a polymer selected from the group consisting of regenerated celluloses, polyesters, polyamides, polyurethanes, polyolefins, acrylonitriles, and any combination thereof.

Clause 13: The method of any preceding Clause, wherein the synthetic polymer comprises polyethylene terephthalate (PET).

Clause 14: The method of any preceding Clause, wherein the synthetic polymer consists essentially of polyethylene terephthalate (PET).

Clause 15: The method of any preceding Clause, wherein the dye-colored synthetic polymer is present in the form of a dye-colored synthetic polymer textile.

Clause 16: The method of any preceding Clause, wherein following the treating, the decolorized synthetic polymer textile has a K/S value of less than 3, as determined using equation (i):

$$K/S = \frac{(1-R)^2}{2R} \quad (i)$$

wherein R=1.0 at 100% reflectance.

Clause 17: The method of any preceding Clause, wherein following the treating, the decolorized synthetic polymer textile has a K/S value as determined using equation (i) which is at least 70% lower than the K/S value of the dye-colored synthetic polymer prior to the treating.

$$K/S = \frac{(1 - R)^2}{2R} \quad (i)$$

wherein R=1.0 at 100% reflectance.

Clause 18: The method of any preceding Clause, wherein a difference between an intrinsic viscosity of the synthetic polymer before and after the treating is less than plus or minus 5%.

Clause 19: The method of any preceding Clause, further comprising a step of pre-soaking the dye-colored synthetic polymer prior to the treating, wherein the pre-soak composition comprises an aqueous solution of an organic solvent.

Clause 20: The method of Clause 19, wherein the organic solvent of the pre-soak composition comprises a ketone.

Clause 21: The method of Clause 20, wherein the organic solvent of the pre-soak composition comprises the same ketone as the treatment composition.

Clause 22: A method for decolorizing a dye-colored polyethylene terephthalate-containing textile, comprising:

- optionally pre-soaking a dye-colored polyethylene terephthalate-containing textile in a presoak composition comprising water and acetone;
- treating the dye-colored textile with a treatment composition, the treatment composition comprising
  - (a) from 2.5 g/L to 50 g/L of sodium formaldehyde sulfoxylate,
  - (b) water, and
  - (d) acetone;

wherein the treatment composition has a pH of 6 or less, and the treating is carried out at a temperature of at least 70° C. and for a duration of time sufficient to at least partially decolorize the dye-colored textile; and

following the treating, separating at least partially decolorized textile from the treatment composition.

Many modifications and other clauses of the disclosure will come to mind to one skilled in the art to which this disclosure pertains having the benefit of the teachings presented in the foregoing descriptions. Therefore, it is to be understood that the disclosure is not to be limited to the specific clauses disclosed herein and that modifications and other clauses are intended to be included within the scope of the appended claims. Although specific terms are employed herein, they are used in a generic and descriptive sense only and not for purposes of limitation. The invention includes any combination of two, three, four, or more of the above-noted clauses as well as combinations of any two, three, four, or more features or elements set forth in this disclosure, regardless of whether such features or elements are expressly combined in a specific clause description herein. This disclosure is intended to be read holistically such that any separable features or elements of the disclosed invention, in any of its various aspects and clauses, should be viewed as intended to be combinable unless the context clearly dictates otherwise.

The invention claimed is:

1. A method for decolorizing a dye-colored synthetic polymer, comprising:

- treating a dye-colored synthetic polymer with a treatment composition, the treatment composition comprising
  - (a) sodium formaldehyde sulfoxylate,
  - (b) water, and
  - (c) a ketone dissolved in the treatment composition;
- wherein the treatment composition has a pH of 6 or less, and the treating is carried out at a temperature of at least

50° C. and for a duration of time sufficient to at least partially decolorize the synthetic polymer; and following the treating, separating at least partially decolorized synthetic polymer from the treatment composition.

2. The method of claim 1, wherein the treatment composition comprises from 2.5 g/L to 50 g/L of sodium formaldehyde sulfoxylate.

3. The method of claim 1, wherein the ketone comprises a ketone selected from the group consisting of acetone, methyl ethyl ketone, 2-pentanone, 3-pentanone, 2-hexanone, 3-hexanone, methyl isobutyl ketone, methyl n-propyl ketone, methyl isopropyl ketone, ethyl ketone, and any combination thereof.

4. The method of claim 1, wherein the ketone comprises acetone.

5. The method of claim 1, wherein the ketone consists essentially of acetone.

6. The method of claim 1, wherein a weight ratio of the water to the ketone in the treatment composition is from 4:1 to 1:4.

7. The method of claim 1, wherein the treating is carried out at a temperature of at least 70° C.

8. The method of claim 1, wherein the ratio of the weight of the treatment composition to the weight of the synthetic polymer during the treating step is at least 10:1.

9. The method of claim 1, wherein the dye-colored synthetic polymer is colored with a dye selected from the group consisting of acridine dyes, anthraquinone dyes, arylmethane dyes, azo dyes, cyanine dyes, nitro dyes, nitroso dyes, phthalocyanine dyes, quinone dyes, thiazine dyes, thiazole dyes, xanthene dyes, fluoresce dyes, stilbene dyes, vinyl sulfone dyes, triazine dyes, sulfur dyes, indigoid dyes, and any combination thereof.

10. The method of claim 1, wherein the dye-colored synthetic polymer material is colored with an azo dye, an anthraquinone dye, or any combination thereof.

11. The method of claim 1, wherein the synthetic polymer comprises a polymer selected from the group consisting of regenerated celluloses, polyesters, polyamides, polyurethanes, polyolefins, acrylonitriles, and any combination thereof.

12. The method of claim 1, wherein the synthetic polymer comprises polyethylene terephthalate (PET).

13. The method of claim 1, wherein the dye-colored synthetic polymer is present in the form of a dye-colored synthetic polymer textile.

14. The method of claim 1, wherein following the treating, the decolorized synthetic polymer textile has a K/S value of less than 3, as determined using equation (i):

$$K/S = \frac{(1 - R)^2}{2R} \quad (i)$$

55 wherein R=1.0 at 100% reflectance.

15. The method of claim 1, wherein following the treating, the decolorized synthetic polymer textile has a K/S value as determined using equation (i) which is at least 70% lower than the K/S value of the dye-colored synthetic polymer prior to the treating

$$K/S = \frac{(1 - R)^2}{2R} \quad (i)$$

65 wherein R=1.0 at 100% reflectance.

16. The method of claim 1, wherein a difference between an intrinsic viscosity of the synthetic polymer before and after the treating is less than plus or minus 5%.

17. The method of claim 1, further comprising a step of pre-soaking the dye-colored synthetic polymer prior to the 5 treating, wherein the pre-soak composition comprises an aqueous solution of an organic solvent.

18. The method of claim 17, wherein the organic solvent of the pre-soak composition comprises a ketone.

19. The method of claim 18, wherein the organic solvent 10 of the pre-soak composition comprises the same ketone as the treatment composition.

20. The method of claim 1, comprising:

optionally pre-soaking a dye-colored polyethylene terephthalate-containing textile in a presoak composition comprising water and acetone;

treating the dye-colored textile with a treatment composition, the treatment composition comprising

(a) from 2.5 g/L to 50 g/L of sodium formaldehyde sulfoxylate,

20

(b) water, and

(c) acetone;

wherein the treatment composition has a pH of 6 or less,

and the treating is carried out at a temperature of at least 70° C. and for a duration of time sufficient to at least 25

partially decolorize the dye-colored textile; and

following the treating, separating at least partially decolorized textile from the treatment composition.

\* \* \* \* \*